

## 1

2,955,034

## AUSTENITIC ALLOY STEEL

Michael Korchynsky and Walter Crafts, Niagara Falls, N.Y., assignors to Union Carbide Corporation, a corporation of New York

No Drawing. Filed Dec. 12, 1958, Ser. No. 779,872 10

7 Claims. (Cl. 75—128)

This invention relates to an austenitic steel alloy possessing a unique combination of mechanical properties.

Current developments in the field of high-temperature materials have been guided by two major considerations. One has been the constantly rising temperatures and stresses that machines and equipment are subjected to and the other is, primarily, a consideration of the economics involved in providing suitable high-temperature materials for use in such machines and equipment.

Presently, there are certain economical austenitic steel alloys in existence capable of withstanding great mechanical stress at high temperature, but the means whereby they are fabricated are limited only to casting since the very structural arrangement of the constituents of the alloy which imparts these high-temperature properties renders them difficult to work. Other austenitic steel alloys have been developed which owe their superior high-temperature properties to a careful working operation, frequently at relatively low temperatures, usually difficult and expensive to accomplish. Such alloys are not suitable for casting.

In contrast to the conventional austenitic steels, the so-called "super alloys," which contain relatively large quantities of cobalt or nickel in addition to chromium and one or more of the elements molybdenum, tungsten, tantalum, and titanium, have the required strength to recommend them for use in the fabrication of machine parts, e.g., blades and other parts of gas turbines, which are subjected to the most severe conditions of stress and temperature. Their use for such a purpose, however, is uneconomical and wasteful of such strategic materials.

For these reasons, it may be seen that there is a need for an austenitic steel alloy (a) possessing good workability, i.e., suitable for use not only in a cast but also in a wrought condition; (b) having a better ability than conventional austenitic steel alloys to withstand severe mechanical stress at higher temperatures; (c) containing less strategic materials than super alloys; and (d) possessing good welding characteristics.

Accordingly, it is an object of this invention to provide an austenitic steel alloy possessing the unique combination of properties set forth above.

Other aims and advantages of the present invention will be apparent from the following description and appended claims.

In accordance with the invention, an austenitic steel alloy is produced that is suitable for use in a wrought and cast condition. This alloy possesses excellent stress resistance properties in extended service at temperatures on the order of 1400° F.

The broad and the preferred compositional ranges from which the critical relationship between the constituent elements of the alloy is established, given in weight percent, are as set forth in Table I below:

## 2

TABLE I

|            | Broad      | Preferred   |
|------------|------------|-------------|
| 5 Chromium | 12 to 25   | 15 to 20.   |
| Manganese  | 10 to 20   | 13 to 17.   |
| Nickel     | 4 to 18    | 8 to 12.    |
| Molybdenum | 2 to 6     | 3 to 5.     |
| Tungsten   | 1 to 4     | 1.5 to 2.5. |
| Nitrogen   | 0.1 to 0.6 | 0.2 to 0.35 |
| Carbon     | up to 0.6  | 0.3 to 0.5  |
| Iron       | Balance    | Balance.    |

The composition of the alloy and the relationship between the constituent elements of the alloy may best be expressed mathematically by the following equation:

$$\frac{y}{x} \leq 1 \leq \frac{y+10}{x}$$

where

$$20 y = 1.6(\text{percent Cr} - 12.5) + 3.5(\text{percent Mo}) + 1.7(\text{percent W}) \quad (\text{A})$$

and

$$x = 20(\text{percent C} + \text{percent N}) + \text{percent Ni} + \frac{1}{3}(\text{percent Mn} - 12) \quad (\text{B})$$

25 In the equation

$$\frac{y}{x}$$

has a value up to and including 1 and

$$\frac{y+10}{x}$$

30 has a value of at least 1 or more. In determining the values of  $y$  or  $x$  to be used in the equation, the weight 35 percent of the elements are substituted in Formulae A and B. These weight percent values are selected from the compositional ranges set forth and the weight percent values selected must satisfy this equation to result in the production of an alloy within the scope of this invention.

40 The subject austenitic steel alloy is capable of withstanding severe mechanical stress at temperatures on the order of 1400° F. At this temperature, the subject austenitic steel alloy has 100- and 1000-hour rupture strengths of at least about 25,000 and 20,000 p.s.i., respectively. In 45 addition, to obtain such an alloy only about 10 percent of the element nickel is necessary in the alloy composition. The following Table II will further illustrate the superior rupture strength properties of the subject alloy as compared with prior austenitic steels and with super alloys.

50 Nickel, one of the alloy constituents, is a well-known extremely effective austenitic stabilizer. However, since it was intended to conserve the strategic material and also reduce the cost of the finished article made therefrom, a manganese-nitrogen combination was used as a substitute for part of the nickel. The alloy base from which the desired properties were obtained was a 15 percent chromium-15 percent manganese-10 percent nickel-balance iron combination.

60 Full use was made of nitrogen as an effective alloy addition, and depending on the manganese plus chromium content, amounts up to 0.6 percent nitrogen were found to be suitable for air-melted alloys and did not result in gas evolution during solidification. Other standard melting procedures may be employed; however, based on economic considerations, air-melting is preferred.

65 With a nitrogen content of about 0.3 percent, a remarkable increase in the rupture strength was produced

TABLE II

Comparison of Cr-Mn-Ni-N austenitic steel of this invention with representative stainless steels and super alloys

RUPTURE STRENGTH AT 1400° F. (P.S.I.)

|                                | 100 Hours | 1,000 Hours | Percent Ni+Co | Percent Fe |
|--------------------------------|-----------|-------------|---------------|------------|
| Cr-Mn-Ni-N                     | 26,000    | 20,000      | 10            | 53.5       |
| Stainless Steels (Austenitic): |           |             |               |            |
| 18Cr-8Ni(304)                  | 10,000    | 6,000       | 8             | 72.0       |
| 18Cr-8Ni-Cb(347)               | 13,000    | 8,000       | 8             | 70.0       |
| 18Cr-8Ni-Mo(316)               | 13,000    | 9,500       | 8             | 67.0       |
| 25Cr-20Ni(310)                 | 15,000    | 8,000       | 20            | 55.0       |
| Super Alloys:                  |           |             |               |            |
| 19-9DL                         | 20,000    | 10,500      | 11            | 63.4       |
| 16-25-6                        | 20,000    | 14,000      | 25            | 48.9       |
| A-286                          | 29,000    | 17,000      | 28            | 50.0       |
| S-590                          | 26,000    | 20,000      | 40            | 26.6       |
| N-155                          | 27,000    | 20,000      | 44            | 24.8       |
| S-816                          | 33,000    | 25,000      | 60            | 5.0 max    |

## COMPOSITION PERCENT

|            | C   | N  | Mn | Cr | Ni | Co | Mo  | W   | Cb/Ta | Ti  | Cu | V | Fe   |
|------------|-----|----|----|----|----|----|-----|-----|-------|-----|----|---|------|
| Cr-Mn-Ni-N | .5  | .3 | 15 | 15 | 10 | —  | 4.0 | 2.0 | —     | —   | —  | — | 53.5 |
| 19-9L      | .3  | —  | 1  | 20 | 11 | —  | 1.5 | 1.5 | 0.5   | 0.8 | .5 | — | 63.4 |
| 16-25-6    | .12 | —  | 2  | 17 | 25 | —  | 7.0 | —   | —     | —   | —  | — | 48.9 |
| A-286      | .08 | —  | 2  | 16 | 28 | —  | 1.5 | —   | —     | 2.0 | .5 | — | 50.0 |
| S-590      | .4  | —  | 1  | 20 | 20 | 20 | 4.0 | 4.0 | 4.0   | —   | —  | — | 26.6 |
| N-155      | .2  | —  | 2  | 22 | 22 | 22 | 3.0 | 3.0 | 3.0   | 1.0 | —  | — | 24.8 |
| S-816      | .4  | —  | 1  | 20 | 20 | 40 | 4.0 | 4.0 | 4.0   | —   | —  | — | 5.0  |

by increasing the carbon content from 0.2 percent to 0.55 percent. It has been found that both the short-time properties and stress-rupture properties increased with increasing increments of carbon. The effect of the carbon content, on the short-time tensile and stress-rupture properties of an iron base alloy containing between about 14.9 and 15.6 percent chromium, 13.8 and 17.6 percent manganese, 10.0 and 10.6 percent nickel, and 0.28 and 0.36 percent nitrogen at 1400° F., is illustrated in Table III below. The yield strength values presented in this table are based on an offset of .2 percent and the elongation values are based on a gauge length of one inch.

TABLE III

Effect of carbon content on the short-time tensile and stress-rupture properties of the Cr-Mn-Ni-N-Fe-base alloy at 1400° F.

| Percent C | Short-Time Properties |                |             | Stress-Rupture Properties at 25,000 p.s.i. |          |             |              |
|-----------|-----------------------|----------------|-------------|--------------------------------------------|----------|-------------|--------------|
|           | Y.S., p.s.i.          | U.T.S., p.s.i. | Percent El. | Percent R.A.                               | Life Hr. | Percent El. | Percent R.A. |
| 0.017     | 24,800                | 34,800         | 5.0         | 4.5                                        | 23.8     | 2.7         | 1.6          |
| 0.14      | 22,200                | 38,200         | 12.0        | 18.8                                       | 42.1     | 5.5         | 6.3          |
| 0.33      | 32,200                | 50,700         | 11.0        | 18.3                                       | 177.6    | 4.2         | 3.3          |
| 0.55      | 38,700                | 55,700         | 42.8        | 55.7                                       | 481.0    | 1.4         | 4.7          |

To the above chromium-manganese-nickel-carbon-nitrogen-iron-base alloy, elements of the group consisting of molybdenum, tungsten, tantalum, columbium, and vanadium were added, separately and in combination, for the purpose of imparting a strengthening effect to the alloy. Of these, a combination of molybdenum plus tungsten proved to be the most effective addition in increasing rupture strength.

The proportions of these two ingredients proved to be critical. The 100- and 1000-hour rupture strength of the steels modified with molybdenum only increased with the increase in the molybdenum content up to 4 percent. Larger amounts of this element, i.e., 6 percent, proved detrimental. The effect of molybdenum on the behavior of steels containing 2 percent tungsten follows, in general, a similar pattern. At 2 percent and 4 percent molybdenum levels, the tungsten-bearing steels were ap-

preciable stronger than the tungsten-free modifications. The drop in strength at the 6 percent molybdenum level was more pronounced in the presence of tungsten. A further increase in the tungsten addition to 4 percent lowered the rupture strength and shifted the optimum molybdenum content to levels below 4 percent.

Rupture tests were conducted on the alloy at 1400° F. In these tests, standard one-quarter inch tensile specimens were used at stresses ranging from 35,000 to 15,000 pounds per square inch to produce rupture times from several hours to over 1000 hours. Stress-rupture tests were also performed, under the same conditions on investment-cast samples of substantially the same composition. The results of these tests are set forth in Table IV below. The yield strength values presented in this table are based on an offset of .2 percent and the elongation values are based on a gauge length of one inch.

TABLE IV

Comparison of high-temperature properties at 1400° F. of a wrought and investment-cast alloy of this invention

| Condition       | Short-Time Properties |              |             | Stress-Rupture Properties at 25,000 p.s.i. |          |             |              |
|-----------------|-----------------------|--------------|-------------|--------------------------------------------|----------|-------------|--------------|
|                 | U.T.S., p.s.i.        | Y.S., p.s.i. | Percent El. | Percent R.A.                               | Life Hr. | Percent El. | Percent R.A. |
| Wrought         | 66,500                | 48,000       | 26.0        | 34.0                                       | 86.9     | 22.6        | 60.3         |
| Investment-Cast | 63,660                | 37,300       | 24.0        | 39.0                                       | 72.7     | 30.0        | 38.5         |

## COMPOSITION PERCENT

|                 | Cr    | Mn    | Ni    | Mo   | W    | C   | N   |
|-----------------|-------|-------|-------|------|------|-----|-----|
| Wrought         | 15.31 | 13.73 | 10.48 | 4.04 | 1.96 | .28 | .28 |
| Investment-Cast | 15.07 | 14.4  | 10.08 | 4.22 | 1.82 | .3  | .32 |

In addition to the unique combination of mechanical properties of the alloy of this invention, it has also been found that the alloy exhibits excellent welding characteristics. The response of the alloy to welding was assessed by means of an annular weld cracking test. The test consists of depositing a weld bead in a circular

groove, machined in a heavy plate. The drastic cooling conditions and the constraint due to the stiffness of the plate create stress inducive to weld cracking. The rate of susceptibility of steel to weld cracking is based on the number of cracks formed during the test, as revealed by visual examination.

The test specimens were machined from a 1-inch thick plate, hot-rolled between 1030 to 1210° C. from a 3-inch by 3-inch air-melted ingot of the following composition, given in weight percent: carbon 0.32, nitrogen 0.37, chromium 15.15, manganese 13.72, nickel 9.77, molybdenum 4.33, and tungsten 2.63. The welding rod was fabricated from the same heat.

An automatic submerged arc electric welding process was used to deposit the annular bead at welding speeds of 22.2 and 34.8 inches per minute.

The resultant weld was free of cracks when deposited at the lower speed of 22.2 inches per minute. At the higher welding speed, two cracks were formed, at the start and at the end of the bead. The results of these two tests were rated excellent and fair, respectively. It should be noted, however, that the higher speed is well in excess of that being used in structural welding of this type of material.

In making the improved subject alloy, a 14 to 16 pound heat was air melted without slag in an induction furnace using a magnesia crucible. The charge consisted of the following virgin materials: technical grade iron, electrolytic nickel, low-nitrogen and high-nitrogen grades of chromium and manganese, nickel-molybdenum master alloy, tungsten powder, and silicon metal. Care was taken not to superheat the melt since an increase in temperature tended to decrease the amount of nitrogen dissolved in the molten steel alloyed with chromium and manganese. The nitrogen addition was made as nitrogen-bearing chromium and manganese at a temperature of about 1550° C., just prior to the final deoxidation with about 0.4 percent silicon.

The heat was cast into 3-inch square split-type cast iron molds. The ingots were forged into one and one-quarter inch square bars, in the temperature range from 1050 to 1250° C. and subsequently rolled to five-eighths inch diameter bars in the same temperature range.

What is claimed is:

1. An austenitic steel alloy suitable for use in a wrought and cast condition, said alloy possessing superior stress resistance properties in extended service at temperatures on the order of 1400° F., said alloy consisting essentially of, by weight percent, 12 to 25 chromium, 10 to 20 manganese, 4 to 18 nickel, 2 to 6 molybdenum, 1 to 4 tungsten, 0.1 to 0.6 nitrogen, up to 0.6 carbon, and the balance iron with incidental impurities, wherein the relationship of the constituent elements in said alloy must satisfy the following equation:

$$\frac{y}{x} \leq | \leq \frac{y+10}{x}$$

where

$$y=1.6(\text{percent Cr}-12.5) + 3.5(\text{percent Mo}) + 1.7(\text{percent W})$$

and

$$x=20(\text{percent C}+\text{percent N}) + \frac{1}{3}(\text{percent Mn}-12)$$

2. An austenitic steel alloy suitable for use in wrought and cast condition and characterized by superior stress resistance properties in extended service at temperatures on the order of 1400° F., said alloy consisting essentially of, by weight percent, 15 to 20 chromium, 13 to 17 manganese, 8 to 12 nickel, 3 to 5 molybdenum, 1.5 to 2.5 tungsten, 0.2 to 0.35 nitrogen, 0.3 to 0.5 carbon, and the balance iron with incidental impurities, wherein the relationship of the constituent elements in said alloy must satisfy the following equation:

$$\frac{y}{x} \leq | \leq \frac{y+10}{x}$$

where

$$y=1.6(\text{percent Cr}-12.5) + 3.5(\text{percent Mo}) + 1.7(\text{percent W})$$

and

$$x=20(\text{percent C}+\text{percent N}) + \frac{1}{3}(\text{percent Mn}-12)$$

3. An austenitic steel alloy suitable for use in the wrought and cast condition and characterized by superior stress resistance properties, in extended service at temperatures on the order of 1400° F., said alloy having a rupture-strength, after 1000 hours under stress at 1400° F., of at least about 20,000 p.s.i., and after 100 hours under stress at 1400° F., of at least about 26,000 p.s.i., said alloy consisting essentially of, by weight percent, 15 to 20 chromium, 13 to 17 manganese, 8 to 12 nickel, 3 to 5 molybdenum, 1.5 to 2.5 tungsten, 0.2 to 0.35 nitrogen, 0.3 to 0.5 carbon, and the balance iron with incidental impurities, wherein the relationship of the constituent elements in said alloy must satisfy the following equation:

$$\frac{y}{x} \leq | \leq \frac{y+10}{x}$$

where

$$y=1.6(\text{percent Cr}-12.5) + 3.5(\text{percent Mo}) + 1.7(\text{percent W})$$

and

$$x=20(\text{percent C}+\text{percent N}) + \frac{1}{3}(\text{percent Mn}-12)$$

4. An austenitic steel alloy suitable for use in the wrought and cast condition, said alloy consisting essentially of about, by weight percent, 15 chromium, 14 manganese, 10 nickel, 4 molybdenum, 2 tungsten, 0.3 nitrogen, 0.3 carbon, and the balance iron with incidental impurities.

5. A structure comprising metal elements welded together, the weld being possessed of superior crack resistance and consisting essentially of, by weight percent, 12 to 25 chromium, 10 to 20 manganese, 4 to 18 nickel, 2 to 6 molybdenum, 1 to 4 tungsten, 0.1 to 0.6 nitrogen, up to 0.6 carbon, and the balance iron with incidental impurities, wherein the relationship of the constituent elements in said alloy must satisfy the following equation:

$$\frac{y}{x} \leq | \leq \frac{y+10}{x}$$

where

$$y=1.6(\text{percent Cr}-12.5) + 3.5(\text{percent Mo}) + 1.7(\text{percent W})$$

and

$$x=20(\text{percent C}+\text{percent N}) + \frac{1}{3}(\text{percent Mn}-12)$$

6. A structure comprising metal elements welded together, the weld being possessed of superior crack resistance and consisting essentially of, by weight percent, 15 to 20 chromium, 13 to 17 manganese, 8 to 12 nickel, 3 to 5 molybdenum, 1.5 to 2.5 tungsten, 0.2 to 0.35 nitrogen, 0.3 to 0.5 carbon, and the balance iron with incidental impurities, wherein the relationship of the constituent elements in said alloy must satisfy the following equation:

$$\frac{y}{x} \leq | \leq \frac{y+10}{x}$$

where

$y = 1.6(\text{percent Cr} - 12.5) + 3.5(\text{percent Mo}) + 1.7(\text{percent W})$   
and

$x = 20(\text{percent C} + \text{percent N}) + \text{percent Ni} + \frac{1}{3}(\text{percent Mn} - 12)$

7. A structure comprising metal elements welded together, the weld being possessed of superior crack re-

sistance and consisting essentially of about, by weight percent, 15 chromium, 14 manganese, 10 nickel, 4 molybdenum, 2 tungsten, 0.35 nitrogen, 0.3 carbon, and the balance iron with incidental impurities.

References Cited in the file of this patent

UNITED STATES PATENTS

|           |          |               |
|-----------|----------|---------------|
| 2,009,974 | Payson   | July 30, 1934 |
| 2,671,726 | Jennings | Mar. 9, 1954  |